

# United States Patent [19]

Ugi et al.

[11] 3,901,708

[45] Aug. 26, 1975

[54] **PROCESS FOR HARDENING LAYERS WHICH CONTAIN GELATIN WITHIN A SILVER HALIDE PHOTOGRAPHIC MATERIAL WITH AN ALDEHYDE AND AN ISONITRILE**

[75] Inventors: **Ivar Ugi, Gruenwald; Heinrich Seibert; Peter Hoffmann**, both of Leverkusen; **Dieter Marquarding, Odenthal-Gloebusch; Harald von Rintelen; Erwin Ranz**, both of Leverkusen; **Wolfgang Himmelmann**, Opladen, all of Germany

[73] Assignee: **Agfa-Gevaert Aktiengesellschaft, Leverkusen, Germany**

[22] Filed: **Apr. 10, 1973**

[21] Appl. No.: **349,764**

[30] **Foreign Application Priority Data**

Apr. 14, 1972 Germany ..... 2218009

[52] U.S. Cl. .... **96/50 PT; 96/111; 260/117; 106/125; 96/51**

[51] Int. Cl. <sup>2</sup> ..... **G03C 5/26; G03C 1/30**

[58] Field of Search ..... 96/111, 50 PT, 50 R, 51; 260/117; 106/125

[56] **References Cited**

**UNITED STATES PATENTS**

|           |         |                    |        |
|-----------|---------|--------------------|--------|
| 2,766,247 | 10/1956 | Middleton.....     | 96/111 |
| 3,295,976 | 1/1967  | Abbott et al.....  | 96/111 |
| 3,554,987 | 1/1971  | Smith.....         | 96/111 |
| 3,701,664 | 10/1972 | Piller et al. .... | 96/111 |

*Primary Examiner*—Won H. Louis, Jr.

*Attorney, Agent, or Firm*—Connolly and Hutz

[57] **ABSTRACT**

A process for hardening layers which contain protein in which the layer is treated with an aldehyde or an aldehyde-donor and with a water soluble, aliphatic or araliphatic isonitrile compound.

**10 Claims, No Drawings**

PROCESS FOR HARDENING LAYERS WHICH  
CONTAIN GELATIN WITHIN A SILVER HALIDE  
PHOTOGRAPHIC MATERIAL WITH AN  
ALDEHYDE AND AN ISONITRILE

This invention relates to a process for hardening layers which contain gelatin, in particular photographic layers.

Many cross-linking agents or hardeners for gelatin have already been described, for example metal salts such as salts of chromium, aluminium or zirconium, aldehydes or their derivatives, in particular formaldehyde, dialdehydes, mucochloric acid, diketones, quinones and chlorides of dibasic organic acids, dianhydrides and in general, compounds which contain several reactive vinyl groups, such as vinyl sulfones and acrylamides. Compounds which contain at least two heterocyclic three membered rings which are easily split, such as ethylene oxide and ethylene imine, may also be used as hardeners for gelatin.

Polyfunctional methanesulfonic acid esters and bis- $\alpha$ -chloroacylamido compounds and derivatives of cyanuric acid chloride and dichloroquinoxaline derivatives have also been described.

High molecular weight hardeners such as polyacrolein and its derivatives or copolymers of alginic acid derivatives have also become known in recent times. There are used particularly as diffusion resistant hardeners which are confined to a particular layer.

Many of the known compounds, however, are not suitable for photographic purposes. Some of them are photographically active while others cannot be used because they have such a deleterious effect on the physical properties of the gelatin layers, e.g. their brittleness. Others again tend to discolour or alter the pH during the hardening reaction. Some cross-linking agents for gelatin also damage the skin, e.g. compounds which contain ethylene imine or ethylene oxide, so that they are unsuitable on physiological grounds. Lastly, for hardeners which are to be used for photographic gelatin layers it is very important, both for the purpose of preparing the layers and for processing them, that one should be able to control the cross-linking reaction within certain limits from the very beginning of the reaction, for example by suitable choice of the drying temperature or of the pH.

In many cases it is desirable in practice to use so-called latent hardeners. By latent hardening is meant a cross-linking reaction which is only fully effective after the material has been subjected to a certain treatment, e.g. the action of alkalies or other factors such as heat. Compounds which are predominantly latent in their action are of great practical importance because the photographic material should not undergo any change while it is stored before it is processed. The reason for this is that the maximum densities obtainable, the  $\gamma$  values and possibly also the light sensitivity of the photographic material decrease with an increasing degree of cross-linking of the layers.

Most of the known hardeners are either too rapid or too slow in their action. If two reactive hardeners are used, e.g. cyanuric acid chloride, the viscosity of the casting solution increases even while the solution is being prepared, before it is cast. In certain casting machines, this causes a constant change in the thickness of the layers. If the hardeners are too slow in their action as is the case, for example, with trisacryloylhex-

ahydrotriazine, the viscosities are not affected and the end points of hardening of the layers are reached only after a prolonged time in storage. All other types of hardeners have properties which are more or less intermediate between those extremes described above.

Processes have already been described in which hardeners which are basically slow in their action are activated by the addition of so-called hardening accelerators. Thus layers which contain trisacryloylhydro-  
10 triazine as hardener can be cross-linked spontaneously by coating them with tertiary amines or alkaline solutions. The photographic properties of these layers, however, often leave much to be desired.

It is an object of this invention to find substances for  
15 hardening layers which contain protein, in particular,  
photographic gelatin layers, which enable the layers to  
be hardened completely within a sufficiently short time  
and which are photographically inert.

It has now been found that this problem can be solved surprisingly simply by hardening the protein layers with an aldehyde or a compound which splits off aldehyde, in the presence of a water-soluble, aliphatic, cycloaliphatic or araliphatic isonitrile compound.

Isonitrile compounds suitable for the process of the invention correspond to the following formulae:



and



in which



*m* = an integer of from 1 to 6,

$$n = 4 \text{ or } 5$$

The following isonitrile compounds have proved to be particularly suitable:

3

|     |                                                                                                                                                                                                     |                               |
|-----|-----------------------------------------------------------------------------------------------------------------------------------------------------------------------------------------------------|-------------------------------|
| 1.  | $\text{CN}-(\text{CH}_2)_m-\text{OCH}_3$                                                                                                                                                            | $m = 2-6$                     |
| 2.  | $\text{CN}-(\text{CH}_2)_m-\text{OC}_2\text{H}_5$                                                                                                                                                   | $m = 2-6$                     |
| 3.  | $\text{CN}-(\text{CH}_2)_m-\text{COONa(K)}$                                                                                                                                                         | $m = 1-6$                     |
| 4.  | $\text{CN}-(\text{CH}_2)_m-\text{OCONH}_2$                                                                                                                                                          | $m = 2-6$                     |
| 5.  | $\text{CN}-(\text{CH}_2)_m-\text{OCON}(\text{CH}_3)_2$                                                                                                                                              | $m = 2,3$                     |
| 6.  | $\text{CN}-(\text{CH}_2)_m-\text{CONH}_2$                                                                                                                                                           | $m = 1-6$                     |
| 7.  | $\text{CN}-(\text{CH}_2)_m-\text{CON}(\text{CH}_3)_2$                                                                                                                                               | $m = 1-6$                     |
| 8.  | $\text{CN}-(\text{CH}_2)_m-\text{CONH}-\text{NH}_2$                                                                                                                                                 | $m = 1-6$                     |
| 9.  | $\text{CN}-(\text{CH}_2)_m-\text{CO}-\text{N} \begin{array}{c} \text{CH}_2-\text{CH}_2 \\ \diagup \quad \diagdown \\ \text{CH}_2-\text{CH}_2 \end{array} \text{O}$                                  | $m = 1-6$                     |
| 10. | $\text{CN}-(\text{CH}_2)_m-\text{N}(\text{CH}_3)_2$                                                                                                                                                 | $m = 2,3$                     |
| 11. | $\text{CN}-(\text{CH}_2)_m-\text{N} \begin{array}{c} \text{CH}_2-\text{CH}_2 \\ \diagup \quad \diagdown \\ \text{CH}_2-\text{CH}_2 \end{array} \text{O}$                                            | $m = 2,3$                     |
| 12. | $\text{CN}-(\text{CH}_2)_3-\text{N} \begin{array}{c} \text{CH}_2-\text{CH}_2 \\ \diagup \quad \diagdown \\ \text{CH}_2-\text{CH}_2 \end{array} \text{N}-\text{CH}_3$                                |                               |
| 13. | $\text{CN}-(\text{CH}_2)_3-\text{N} \begin{array}{c} \text{CH}_2-\text{CH}_2 \\ \diagup \quad \diagdown \\ \text{CH}_2-\text{CH}_2 \end{array} \text{N}-(\text{CH}_2)_3-\text{CN}$                  |                               |
| 14. | $\begin{array}{c} \text{CH}_2-\text{CH}_2 \\ \diagup \quad \diagdown \\ \text{CH}_2-\text{CH}_2 \end{array} \text{C} \begin{array}{c} \text{NC} \\ \diagup \quad \diagdown \\ \text{y} \end{array}$ | $y = \text{COONa(K)}$         |
| 15. | $\text{Y} = \text{CONH}$                                                                                                                                                                            |                               |
| 16. | $\text{Y} = \text{CONH}-\text{NH}_2$                                                                                                                                                                |                               |
| 17. | $\text{Y} = \text{CO}-\text{N}(\text{CH}_3)_2$                                                                                                                                                      |                               |
| 18. | $\text{Y} = \text{CO}-\text{N} \begin{array}{c} \text{CH}_2-\text{CH}_2 \\ \diagup \quad \diagdown \\ \text{CH}_2-\text{CH}_2 \end{array} \text{O}$                                                 |                               |
| 19. | $\begin{array}{c} \text{CH}_2-\text{CH}_2 \\ \diagup \quad \diagdown \\ \text{CH}_2-\text{CH}_2 \end{array} \text{C} \begin{array}{c} \text{NC} \\ \diagup \quad \diagdown \\ \text{Y} \end{array}$ | $\text{Y} = -\text{COONa(K)}$ |
| 20. | $\text{Y} = -\text{CONH}_2$                                                                                                                                                                         |                               |
| 21. | $\text{Y} = -\text{CONH}-\text{NH}_2$                                                                                                                                                               |                               |
| 22. | $\text{Y} = -\text{CO}-\text{N}(\text{CH}_3)_2$                                                                                                                                                     |                               |
| 23. | $\text{Y} = -\text{CO}-\text{N} \begin{array}{c} \text{CH}_2-\text{CH}_2 \\ \diagup \quad \diagdown \\ \text{CH}_2-\text{CH}_2 \end{array} \text{O}$                                                |                               |
| 24. | $\begin{array}{c} \text{CH}_2-\text{CH}_2-\text{NC} \\   \\ \text{CH}_2-\text{CH}_2 \\   \\ \text{S} \\ \diagup \quad \diagdown \\ \text{O}_2 \end{array}$                                          | 50                            |
| 1.  | $\begin{array}{c} \text{CH}_2-\text{CH}-\text{NC} \\   \\ \text{CH}_2-\text{CH}_2 \\   \\ \text{SO}_2 \end{array}$                                                                                  | 55                            |

60

## 3-Isocyanosulpholan

171.5 g of 3-Aminosulfolan hydrochloride and 77 g of sodium formate are suspended in a mixture of 500 ml of benzene and 200 ml of formic acid and heated to boiling. After quantitative removal of the water which separates, the solution is concentrated by evaporation

under vacuum. The dark brown residue is dissolved in 1000 ml of methylene chloride and 252 g of triethylamine, and 91 ml of phosgene are introduced into this solution at a temperature of about 35°C with stirring. Stirring is then continued for 15 minutes, ammonia is introduced at 10°C until the solution is saturated with ammonia, and the precipitate is then filtered off. The fil-

trate is concentrated by evaporation under vacuum at a bath temperature of 35°C. The residue is filtered over silica gel (benzene/ethyl acetate 1:1) and charcoal (methanol) and recrystallised from methanol.

Yield: 80 g (55% of the theory), m.p. 94°–94.5°C.  
 $C_5H_7NO_2S$  (145) Calculated: C 41.30; H 4.83; N 9.66; S 22.05; Found: C 41.3; H 4.9; N 9.8; S 21.8

## II. $CN-(CH_2)_3-CH_2-OCH_3$

### 2-Isocyano-1-methoxy-ethane

94 g of 2-N-formylamino-1-methoxy-ethane are dissolved in 200 ml of methylene chloride and 200 ml of triethylamine. 100 g of phosgene are then introduced. After stirring for 15 minutes, the solution is saturated with gaseous ammonia at 10°C, the precipitate is suction filtered and the filtrate is concentrated by evaporation under vacuum (bath temperature 20°C) and the residue is distilled under vacuum.

Yield: 29 g (37.5% of the theory) b.p. 18 mm 50°C. The CO-isocyano-1-methoxy-alkanes and -ethoxy-alkanes  $CN-(CH_2)_n-OR$  ( $N=2-6$ ; R =  $-CH_3$ ,  $-C_2H_5$ ) are prepared in analogous manner.



### N,N-Bis-1-(3-isocyano-propyl)-piperazine

343 g of N,N-Bis-1-(3-N-formylaminopropyl)-piperazine are dissolved in 1750 ml of methylene chloride and 870 ml of triethylamine, and 272 g of phosgene are introduced at 10 to 15°C with vigorous stirring. Stirring is then continued for 10 minutes and the solution is then saturated with gaseous ammonia at 10°C. The precipitate is suction filtered and washed thoroughly with methylene chloride. The filtrate is distilled off under vacuum at a bath temperature of 30°–35°C and the residue is recrystallised from methanol.

Yield: 230 g (75% of the theory), m.p. 80°–81°C.

N-Methyl-N-1-(3-isocyano)-piperazine is prepared in analogous manner.



### 3-Isocyano-1-(N-morpholino)-propane

1316 g of 3-Amino-1-(N-morpholino)-propane are introduced dropwise into 1500 g of methyl formate with vigorous stirring and the mixture is then heated to boiling for 10 hours. The volatile constituents are removed under vacuum (water pump) at a bath temperature of 75°C. The oily residue is dissolved in 4500 ml of methylene chloride and 2805 ml of triethylamine, and 877 g of phosgene are introduced at 35°C with stirring. The reaction mixture is cooled to 5°C and 300 to 350 g of ammonia are introduced. The reaction mixture is then filtered and the filtrate concentrated by evaporation under vacuum (water pump) at 50°C. The residue is distilled.

B.p. 72°–73°C/0.25 mm Hg, yield: 1100 g (82% of the theory)

$C_8H_{11}N_2O$  (154) Calculated: C 62.31; H 9.15; N 18.17; O. 10.38; Found: C 62.6; H 9.6; N 18.0; O. 10.5



5 and  $CN-(CH_2)_n-N(CH_3)_2$  ( $n=2, 3$ ) are prepared in analogous manner.

## V. $CN-(CH_2)_3-COO Na$

### 10 Sodium salt of $\gamma$ -isocyanobutyric acid

70.0 g of the hydrochloride of methyl  $\gamma$ -aminobutyrate were suspended in 280 ml of methylene chloride and then heated to boiling after the addition of 250 ml of methyl formate. 49 g of triethylamine are then added dropwise with stirring and after 10 hours the reaction mixture is cooled to 5°C. The precipitate is suction filtered and the filtrate is concentrated by evaporation under vacuum at a bath temperature 40°C. The residue is dissolved in 250 ml of methylene chloride and 110 ml of triethylamine, and 38 g of phosgene are introduced at 30°–40°C with stirring. The reaction is left to continue for 10 minutes and the reaction mixture is then saturated with ammonia at 10°C, the precipitate is suction filtered, the filtrate is concentrated by evaporation under vacuum and the residue is distilled under vacuum.

25 25.4 g of methyl  $\gamma$ -isocyanobutyrate (b.p. 0.35 mm = 67°–75°C) are obtained, which are then introduced dropwise into 110 ml of 2N sodium hydroxide solution at 10°C with stirring. After leaving the reaction mixture to stand at room temperature for 24 hours, it is concentrated by evaporation under vacuum at a temperature of up to 30°C. The solid residue is washed with benzene and recrystallised from methanol.

30 35 Yield: 26 g (42.5% of the theory), m.p. 156°–159°C.  
 The sodium salts  $CN-(CH_2)_n-COO Na$  ( $n=1, 2, 4, 5, 6$ ) are prepared in analogous manner.

## VI. $CN-(CH_2)_5-COOK$

### 40 Potassium salt of 6-isocyano-caproic acid

98 g of the hydrochloride of ethyl 6-aminocaproate are suspended in 300 ml of methylene chloride and covered with a solution of 106 g of soda in 200 ml of water. A mixture of 75 mol of 98% formic acid and 63 ml of acetic anhydride which has previously been left to stand for one-half hour is introduced dropwise with vigorous stirring. The reaction mixture is left to react for 1 hour and the aqueous phase is then separated off.

45 50 Concentrated aqueous soda solution is added to the organic phase until the pH is 7.5 to 9 (controlled by pH meter) and the organic phase is cooled to 0° to 5°C. 80 g of phosgene are then introduced and at the same time concentrated sodium hydroxide solution is added dropwise to maintain the pH constantly between 7.5 and 9. After 1 hour, 170 ml of water are added and the organic phase is separated off, dried and concentrated by evaporation under vacuum. The residue is distilled.

55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695

VII.  $\text{CN}-\text{CH}_2\text{CO}-\text{NH}_2$ 

## Isocyno acetic acid amide

10 g of ethyl isocynoacetate [I. Ugi et al, Angew. Chem. 77, 492 (1965)] are dissolved in 50 ml of ethanol and the solution is cooled to 0° to 5°C. A catalytic quantity of sodium methoxide is added and ammonia is introduced for 1 hour. The clear solution is concentrated by evaporation under vacuum at room temperature and the solid residue is washed with a small quantity of cold propanol and ether and suction filtered. Yield: 5 g (83% of the theory), m.p. 121°-122°C.

VIII.  $\text{CN}-(\text{CH}_2)_2-\text{CONH}_2$  $\gamma$ -Isocyanobutyric acid amide

30 g of methyl  $\gamma$ -isocyanobutyrate are dissolved in 100 ml of methanol, and ammonia is then introduced for one hour without cooling. The temperature rises to about 45°C. The reaction mixture is left to stand at room temperature for 3 days and then concentrated by evaporation under vacuum. The residue is recrystallised from ethyl acetate.

Yield: 13 g (50% of the theory), m.p. 64°-65°C.

$\text{C}_2\text{H}_8\text{N}_2\text{O}$  (112) Calculated: C 53.55; H 7.19; N 24.99;

Found: C 53.7; H 7.4; N 24.6

The compounds

$\text{CN}-(\text{CH}_2)_n-\text{CONH}_2$  ( $n = 2, 4, 5, 6$ ) and

$\text{CN}-(\text{CH}_2)_n-\text{CON}(\text{CH}_3)_2$  ( $n = 1-6$ )



are prepared in analogous manner.

IX.  $\text{CN}-\text{CH}_2-\text{CO}-\text{NH}-\text{NH}_2$ 

## Isocyno-acetic acid hydrazide

10 g of ethyl isocynoacetate [I. Ugi et al, Angew. Chem. 77, 492 (1965)] are dissolved in 40 ml of ethanol. After cooling to 0°C, 5 g of hydrazine hydrate are introduced dropwise and the reaction mixture is stirred at 0°C for 1 hour. The crystalline product is then suction filtered and washed with a little cold ethanol and ether.

Yield: 7.8 g (89% of the theory) m.p. 92°-93°C.

The hydrazides  $\text{CN}-(\text{CH}_2)_n-\text{CO}-\text{NH}-\text{NH}_2$  ( $n = 2-6$ ) are prepared in analogous manner.



## Sodium salt of 1-isocyno-cyclohexane carboxylic acid-(1)

46 g of N-formyl-1-amino-1-carbomethoxycyclohexane are dissolved in 250 ml of ethylene chloride and 83 ml of triethylamine, and 25 g of phosgene are introduced at 30°-40°C. The reaction mixture is then stirred for 15 minutes and washed, first with a saturated sodium bicarbonate solution and then with water. The organic phase is dried and concentrated by evaporation under vacuum. The residue is distilled (b.p. 0.03 mm 50°C) and dissolved in 110 ml of 2N sodium hydroxide solution, the temperature rising to about 40°C. After stirring this solution for 1 hour, it is concentrated by evaporation under vacuum.

Yield: 36.6 g (77% of the theory), m.p. 320°-323°C (decomposition).

The sodium salt of 1-isocyno-cyclopentane carboxylic acid-(1) is prepared in analogous manner.

The compounds



are prepared from the methyl or ethyl esters



35 The light sensitive emulsion layers for which the hardening process according to the invention is particularly suitable are, for example, those layers which are based on non-sensitized emulsions, orthochromatic, panchromatic or infra-red emulsions, X-ray emulsions and other emulsions which are not spectrally sensitized.  
 40 The hardening process according to the invention has also proved suitable for hardening gelatin layers used for various black-and-white photographic processes and colour photographic processes. The process according to the invention has proved particularly advantageous for hardening composite photographic layers used for colour photographic processes, e.g. those which contain emulsion layers with colour couplers or emulsion layers which are designed to be treated with  
 45 solutions which contain colour couplers.

50 55 The aldehydes and isonitrile compounds may also be added at separate stages in the process according to the invention without the effect of the combination being thereby lost. Thus, for example a gelatin layer having a melting point of 50° to 60°C (to be defined hereinafter) may be prepared with the addition of isonitrile, and the aldehyde component may subsequently be added to this gelatin layer by bathing the layer in an aqueous solution of the component before the material is processed. The melting point of the layer then increases considerably, and hence also the degree of hardening.  
 60 65 It is also immaterial in principle whether the isonitrile and aldehyde compounds are used together in one layer or in separate layers or whether the second com-

ponent is poured over the top as an aqueous solution, provided that one of the two compounds is diffusible. The hardening action sets in at once when the two components meet in a layer which consists of a protein or, as in the present case, of gelatin.

The hardening of photographic gelatin layers by the process according to the invention can therefore be achieved either by using the aldehyde and isonitrile compound in the same or different layers of a photographic material or by adding the compounds to preliminary and/or after-hardening baths. With this method, the photographic material may be treated either before or after the photographic process either with separate baths for the aldehyde compounds and for the isonitrile compound or with baths which contain the two compounds together.

According to the invention, the aldehydes are used in quantities of 0.1 to 8% by weight, based on gelatin, and preferably in quantities of 0.5 to 7% by weight, and the isonitrile compounds are used in quantities of 0.05 to 15% by weight and preferably in quantities of 0.1 to 10% by weight.

The usual silver halide emulsions are suitable for the hardening process described here. The silver halide contained in them may be silver chloride, silver bromide or mixtures thereof, optionally with a small silver iodide content, i.e. up to 20 mols percent. Photographic materials prepared with these emulsions may contain the emulsion layers either as single layers, e.g. in the case of simple black-and-white materials, or as several layers arranged above one another, e.g. in the case of colour photographic materials. Each of the individual layers of these layer combinations may contain the usual additives.

The binders used for the photographic layers are protein layers, preferably gelatin although gelatin may be partly replaced by other natural or synthetic binders. Suitable natural binders are e.g. alginic acid and its derivatives such as salts, esters or amides, cellulose derivatives such as carboxymethyl cellulose, alkyl cellulose such as hydroxyethyl cellulose, starch or derivatives of starch such as ethers or esters or carrageenates. Suitable synthetic binders are: polyvinyl alcohol, partly saponified polyvinyl acetate, polyvinyl pyrrolidone and the like.

The emulsions may also be chemically sensitized, e.g. by the addition of sulphur compounds during the stage of chemical ripening, for example allyl isothiocyanate, allyl thiourea, sodium thiosulfate, etc.. The chemical sensitizers used may also be reducing agents, e.g. the tin compounds described in Belgian Pat. Nos. 493,464 and 568,687, polyamines such as diethylene triamine or aminomethylsulfonic acid derivatives, e.g. according to Belgian Pat. No. 547,323.

Noble metals such as gold, platinum, palladium, iridium, ruthenium or rhodium or compounds of these metals are also suitable chemical sensitizers. This method of chemical sensitization has been described in the article by R. Koslowski, Z. Wiss. Phot. 46, 65-72 (1951).

The emulsions may also be sensitized with polyalkylene oxide derivatives, e.g. with polyethylene oxide having a molecular weight of between 1000 and 20,000, or with condensation products of alkylene oxides and aliphatic alcohols, glycols, cyclic dehydration products of hexitols, alkyl substituted phenyls, aliphatic carboxylic acid, aliphatic amines, aliphatic diamines and amides.

The condensation products have a molecular weight of at least 700 and preferably more than 1000. These sensitizers may, of course, also be combined to achieve special effects, as described in Belgian Pat. No. 537,278 and in British Pat. No. 727,982.

The emulsions may also be optically sensitized, e.g. with the usual polymethine dyes such as neutrocyanine, basic or acid carbocyanines, rhodacyanines, hemicyanines, styryl dyes, oxonoles and the like. Sensitizers of this kind have been described in the work by F. M. Hammer "The Cyanine Dyes and related Compounds", (1964).

The emulsions may contain the usual stabilizers, e.g. homopolar or salt-type compounds of mercury which contain aromatic or heterocyclic rings, such as mercaptotriazoles, simple mercury salts, sulfonium mercury double salts and other mercury compounds. Azaindenes, especially tetra- or penta-azaindenes and particularly those which are substituted with hydroxyl or amino groups are also suitable stabilizers. Compounds of this type have been described in the article by Birr, Z. Wiss. Phot. 47, 2-58 (1952). Other suitable stabilizers are inter alia heterocyclic mercapto compounds, e.g. phenylmercaptotetrazole, quaternary benzothiazole derivatives, benzotriazole and the like.

The emulsions may also contain the usual additives used for colour photographic materials, e.g. colour couplers.

The activity of the hardener combination according to the invention may be demonstrated in known manner by measuring the melting point of the layers or degree of swelling of the layers.

The melting point of the layers is determined as follows: The layer cast on a support is half dipped into water which is continuously heated to 100°C. The temperature at which the layer runs off the support (formation of streaks) is taken as the melting point or melting off point. If no melting occurs at temperatures up to 100°C, the layer is again kept at 100°C for a maximum of 30 minutes. The measure of the hardening in that case is the length of time after which the layer runs off the support. Under the conditions of measurement, pure gelatin layers without hardener show a melting off point of 30° - 35°C.

Swelling is determined gravimetrically after 10 minutes treatment in distilled water at 22°C and is indicated in percent.

#### EXAMPLE 1

A gelatin-containing silver chlorobromide emulsion which is composed of 80 g of gelatin, 38 g of silver nitrate in the form of the halides and 0.5% of glyoxal (based on the quantity of gelatin) per kg of solution is cast on a layer support of triacetyl cellulose at pH 6.2 and dried. The material is then divided into 3 parts A, B and C. Part B is coated with the following mixture:

500 cc of a 2% aqueous gelatin solution and  
4 ml of a 1% solution of compound II.

Part C is coated with a mixture of

500 ml of a 2% aqueous gelatin solution and  
4 ml of a 1% solution of compound I in a 1:3 mixture  
of dimethylformamide/H<sub>2</sub>O.

After drying, the melting points of the samples are determined immediately and after 1 hour, 2 hours and 3 hours storage. The results are summarized in the table below:

## 11

Table 1

| Sample | Melting point after storage of the layers at room temperature in °C |    |    |    |       |
|--------|---------------------------------------------------------------------|----|----|----|-------|
|        | 0                                                                   | 1  | 2  | 3  | hours |
| A      | 58                                                                  | 58 | 58 | 58 |       |
| B      | 62                                                                  | 65 | 69 | 74 |       |
| C      | 57                                                                  | 72 | 73 | 78 |       |

The figures show that the hardening effect of the combination of aldehyde and isonitrile compound is greater than that of aldehyde alone.

## EXAMPLE 2

A 3% aqueous gelatin solution which contains 0.2% of formalin, based on the weight of gelatin, is cast as an NC layer on a triacetyl cellulose support which has been prepared on both sides. After drying and 24 hours storage at room temperature with exclusion of moisture, the layer has a melting point of 47°C. It is then bathed for 2 minutes in a 1% aqueous solution of compound II and washed for 10 minutes. After this treatment, the melting point of the layer has risen to 75°C.

## EXAMPLE 3

An aqueous silver chlorobromide emulsion which contains gelatin and is composed of 80 g of gelatin, 40 g of silver nitrate in the form of the halides and 0.4% of formalin based on the dry weight of gelatin) per kg of mixture (pH 6.2) is cast on a layer support of ethylene terephthalate (Sample A). Half of the mixture cast on the support is covered with a top layer consisting of a 2% aqueous solution of compound X (at pH 5.6) (Sample B). The melting points of the layer were determined immediately after drying and after 1,2,3,24 and 40 hours storage at room temperature. The results shown in the following table are obtained:

Table 2

| Sample | Melting points after storage at room temperature with exclusion of moisture in °C |      |      |      |      |        | Vertical swelling after 10 minutes washing at 22°C |
|--------|-----------------------------------------------------------------------------------|------|------|------|------|--------|----------------------------------------------------|
|        | 0                                                                                 | 1    | 2    | 3    | 24   | 40 hrs |                                                    |
| A      | 45°                                                                               | 55°  | 62°  | 72°  | 93°  | 95°    | 395%                                               |
| B      | 100°                                                                              | 100° | 100° | 100° | 100° | 100°   | 310%                                               |

As shown in the last column of the table, the addition of compound I also reduces the swelling of the layer as a whole.

## EXAMPLE 4

100 ml portions of gelatin-containing silver chlorobromide emulsions which contain 100 g of gelatin and 40 g of silver nitrate in the form of the halides per kg of emulsion are treated with the following additives:

Sample A: 0.3% of formalin, based on the gelatin content (in the form of a 1% solution),

Sample B: 0.3% of compound I (in the form of a 1% solution),

Sample C: 0.3% of formalin and 0.3% of compound I,

Sample D: 0.3% of compound V (in the form of a 1% solution),

Sample E: 0.3% of formalin and 0.3% of compound V.

## 12

The samples are adjusted to pH 6.2 and cast on a layer support of cellulose acetate. The melting points of the layers are determined immediately after drying and after 1,2,3,4 and 5 hours storage. The following results are obtained:

Table 3

| Sample | Melting points after storage at room temperature with exclusion of moisture in °C |     |     |     |       |       | hrs. |
|--------|-----------------------------------------------------------------------------------|-----|-----|-----|-------|-------|------|
|        | 0                                                                                 | 1   | 2   | 3   | 4     | 5     |      |
| A      | 39                                                                                | 43  | 48  | 48  | 48-56 | 60-84 |      |
| B      | 37                                                                                | 37  | 37  | 37  | 37    | 37    |      |
| C      | 100                                                                               | 100 | 100 | 100 | 100   | 100   |      |
| D      | 37                                                                                | 37  | 37  | 37  | 37    | 37    |      |
| E      | 38                                                                                | 50  | 56  | 64  | 80    | 90    |      |

The results show that the isonitrile compounds alone have no hardening effect and that mixtures of formalin with isonitriles are more powerful hardeners than formalin alone.

## EXAMPLE 5

An emulsion layer of the following composition is applied to a layer support of baryta paper:

200 ml of a silver bromide gelatin emulsion containing

3% by weight of silver halide and 6% by weight of gelatin,

4.4 ml of a 10% aqueous solution of saponin, and 0.34 ml of a 30% aqueous solution of formaldehyde.

This is coated with a gelatin solution of the following composition:

200 ml of a 2% aqueous gelatin solution,

4 ml of a 5% solution of compound III in a 3:1 mixture of water/dimethylformamide, and

4 ml of a 10% aqueous solution of saponin.

The whole layer contains 2.0 g of silver nitrate per m<sup>2</sup> in the form of silver bromide and 0.07 g of compound III, the top layer having a thickness of about 1 m $\mu$ .

After 24 hours storage at room temperature, the

40

35

30

25

20

15

10

5

0

40

35

30

25

20

15

10

5

0

40

35

30

25

20

15

10

5

0

40

35

30

25

20

15

10

5

0

40

35

30

25

20

15

10

5

0

40

35

30

25

20

15

10

5

0

40

35

30

25

20

15

10

5

0

40

35

30

25

20

15

10

5

0

40

35

30

25

20

15

10

5

0

40

35

30

25

20

15

10

5

0

40

35

30

25

20

15

10

5

0

40

35

30

25

20

15

10

5

0

40

35

30

25

20

15

10

5

0

40

35

30

25

20

15

10

5

0

40

35

30

25

20

15

10

5

0

40

35

30

25

20

15

10

5

0

40

35

30

25

20

15

10

5

0

40

35

30

25

20

15

10

5

0

40

35

30

25

20

15

10

5

0

40

35

30

25

20

15

10

5

0

40

35

30

25

20

15

10

5

0

40

35

30

25

20

15

10

5

0

40

35

30

25

20

15

10

5

0

40

35

30

25

20

15

10

5

0

40

35

30

25

20

15

10

5

0

40

35

30

25

20

15

10

5

0

40

35

30

25

20

15

10

5

0

40

35

30

8 ml of a 5% aqueous solution of compound VII. This is coated with a gelatin solution of the following composition:

200 ml of a 2% aqueous gelatin solution,  
20 ml of a 5% aqueous succinic dialdehyde,  
4 ml of a 10% aqueous solution of saponin.

The whole layer contains 1.5 g of silver nitrate per m<sup>2</sup> in the form of silver chloride and about 0.6 g of compound VII, and the thickness of the top layer is about 1  $\mu$ .

After 24 hours storage at room temperature, the layer combination is not dissolved after 18 minutes in boiling water.

#### EXAMPLE 7

A black-and-white photographic paper which has been only slightly hardened and is not sufficiently resistant for drying on a drying drum is treated for 2 minutes with a bath of the following composition after the developed and fixed image has been bathed in water:

90 ml of water,  
5 ml of compound IV  
2.5 ml of a 30% aqueous solution of formaldehyde.

A material which is very resistant on the drying drum is obtained in this way.

#### EXAMPLE 8

Emulsion layers which have not been hardened and which contain 80 g of gelatin and 38 g of silver nitrate in the form of the halides are treated with the following freshly prepared prehardening baths (3 minutes, 20° to 22°C) before development:

##### Prehardening bath I

550 ml of water  
154 g of sodium sulfate  
20 g of sodium acetate  
16.6 ml of 30% aqueous solution of formaldehyde made up to 1000 ml with water.

##### Prehardening bath II

A. 550 ml of water  
154 g of sodium sulfate  
20 g of sodium acetate  
16.6 ml of 30% aqueous solution of formaldehyde  
5 g of compound I  
made up to 1000 ml with water

B. the same as A, but

10 g of compound I

##### Prehardening bath III

A. 550 ml of water  
154 g of sodium sulfate  
20 g of sodium acetate  
16.6 ml of 30% aqueous solution of formaldehyde  
5 g of compound II  
made up to 1000 ml with water

B. the same as A., but

10 g of compound II

The layers are then washed for 10 minutes and dried before determination of the melting point. The following results are obtained:

| Prehardening bath | Melting point of the layer in °C | 65    | II |
|-------------------|----------------------------------|-------|----|
| I                 | 43                               |       |    |
| II A              | 10°                              | 100°C |    |
| II B              | 10°                              | 100°C |    |
| III A             | 10°                              | 100°C |    |

-Continued

|   | Prehardening bath | Melting point of the layer in °C |
|---|-------------------|----------------------------------|
| 5 | III B             | 10° 100°C                        |

\*The layer becomes detached from its support after 10 minutes in boiling water.

The figures show that the quantity of formalin used is not sufficient on its own to cross-link the gelatin layers so that they become resistant to boiling. A high degree of cross-linking is obtained only when the isonitriles are also added.

15

#### EXAMPLE 9

The use of the prehardening bath described in Example 8 is modified as follows.

20 A slightly hardened layer combination of a colour reversal material prepared in accordance with Fiat Final Report 943, pages 14 and 15, is treated successively with prehardening baths of the following composition, in each case for 3 minutes at 20° to 22°C:

##### Bath A

550 ml of water,  
154 g of sodium sulfate  
20 g of sodium acetate  
16.6 ml of 30% aqueous solution of formaldehyde made up to 1 l with water.

##### Bath B

550 ml of water  
154 g of sodium sulfate  
20 g of sodium acetate  
10 g of compound I

made up to 1 l with water.

The material is washed for 10 minutes and then dried. After this prehardening process, it was found to melt off at temperatures above 100°C (boiling time more than 10' at 100°C).

40 The same results were obtained with compounds IV, V and VI instead of compound I.

A sample which was treated with Bath A alone was found to have a melting point of 43°C.

45 The same results were obtained when emulsion layers were treated with after-hardening baths by a treatment corresponding to Examples 8 and 9.

What we claim is:

1. A process for hardening a photographic material comprising photographically processing a photographic material containing on a support a layer containing a protein compound and a silver halide emulsion layer, or a layer of a silver halide emulsion containing a protein compound wherein the improvement comprises treating the photographic material in a step which contains an aldehyde or an aldehyde-donor compound and an isonitrile compound selected from the group consisting of a watersoluble, isonitrile compound of the following formula

60 I



or



in which

$R_1$  is  $-\text{OCH}_3$ ,  $-\text{OC}_2\text{H}_5$ ,  $-\text{OCONH}_2$ ,  $-\text{OCON}(\text{CH}_3)_2$ ,  $-\text{CONH}_2$ ,  $-\text{N}(\text{CH}_3)_2$ ,



$R_1$  or  $R_2$  is  $-\text{COONa(K)}$ ,  $-\text{CON}(\text{CH}_3)_2$ ,  $-\text{CONH}-\text{NH}_2$ ,  $-\text{CONH}_2$



$m$  is an integer of from 1 to 6,

$n$  is 4 or 5.

2. A process as claimed in claim 1 in which before the photographic material is photographically processed said protein-containing layer is successively treated with two prehardening baths, one of which contains

35

40

45

50

55

60

said aldehyde compound and the other said isonitrile compound.

3. A process as claimed in claim 1 in which after the photographic material has been photographically processed, the protein-containing layer is treated with an after-hardening bath which contains said aldehyde compound and said isonitrile compound.

4. A process as claimed in claim 1 in which the layer which is to be hardened is of a photographic material and after the material is photographically processed, the layer to be hardened is successively treated with two after-hardening baths, one of which contains said aldehyde compound and the other said isonitrile compound.

15 5. A process as claimed in claim 1 in which said photographic material consists of a plurality of gelatin-containing layers.

6. A process as claimed in claim 4 in which gelatin is hardened in a multilayered color photographic material.

7. A product according to the process of claim 1.

8. A process as claimed in claim 1 in which the protein-containing layer to be hardened contains one of the treating agents and the other agent is contained in a treatment bath.

9. A process as claimed in claim 1 in which the protein-containing layer to be hardened contains both of said treating agents.

30 10. A process as claimed in claim 1 in which the protein-containing layer to be hardened contains one of the treating agents and the silver halide emulsion layer contains the other treating agent.

\* \* \* \* \*